

## UNITED STATES PATENT OFFICE

2,028,257

## MINERAL OIL COMPOSITION

Bertrand W. Story, Paulsboro, and Everett W. Fuller, Woodbury, N. J., assignors to Socony-Vacuum Corporation, New York, N. Y., a corporation of New York

No Drawing. Application September 7, 1933,  
Serial No. 688,436

1 Claim. (Cl. 87—9)

This invention relates to the improvement of viscous oils, such as turbine oils and insulating oils, which have been highly refined, as by the use of large quantities of sulphuric acid, including fuming acid. Such highly refined oils are susceptible, under the elevated temperatures encountered in their use, to atmospheric oxidation resulting particularly in the formation of coloring matter and acid. The purpose of the invention is to produce compositions, for such oils, in which such color and acid formation is greatly reduced or substantially inhibited.

In our application for Letters Patent of the United States, filed June 10, 1931, Serial No. 543,396, we have disclosed the discovery that dibenzyl disulfide has the capability of inhibiting, to a large extent, the formation of acid in highly refined oils when dissolved therein in small quantities. In his application for Letters Patent of the United States filed February 16, 1933, Serial No. 657,106, the applicant Fuller has shown that the monosulfides of hydroxy aromatic compounds have the same capability. We have now discovered that the use, in combination with dibenzyl disulfide of a monosulfide of a hydroxy-aromatic compound results in the inhibition of color and acid formation, in highly refined viscous oils, to a degree much beyond that which can be attained by the use of either stabilizing body alone in its optimum quantity. As an example, taken from the results hereinafter tabulated, it has been found that in a given oil subjected to an oxidation test, in the presence of copper foil, for 96 hours, the acid value, (neutralization number), using 0.05% of dibenzyl disulfide alone, was 0.13, and using 0.010% of monosulfide of m-cresol, was 6.05. By the use of 0.05% of dibenzyl disulfide, together with either 0.010% or 0.005% of monosulfide of m-cresol, the acid value was reduced to 0.02; that is, to less than one sixth of that occurring with the dibenzyl disulfide alone, and less than one three-hundredth of that occurring with the monosulfide of m-cresol alone. The color, with the dibenzyl disulfide alone, was 13 and with the 0.10% of monosulfide of m-cresol alone it was 14, but with the two materials used together the color was reduced to 1.

We give hereinafter, in tabular form, the results of tests of dibenzyl disulfide and of various monosulfides of hydroxy aromatic compounds, in various quantities and for various periods, both alone and in combination.

In each of the tests in question a 200 gram sample of the oil, containing a piece of freshly polished copper foil 40 x 70 x 0.1 millimeters in size, was maintained at a temperature of 120° C. while oxygen gas was bubbled through it at the rate of 2,000 ml. per hour. 10 ml. samples of the oil

were tested, after the indicated time intervals, for Lovibond color and neutralization number.

Example 1.—Transformer oil, consisting of Coastal distillate treated with 50 lbs. of 98% sulphuric acid and 200 lbs. of 104% sulphuric acid per barrel of oil, neutralized with sodium hydroxide and filtered through fuller's earth. Its color, Lovibond, was less than 0.1, specific gravity 0.870; viscosity, Saybolt universal at 100° F., 69 seconds.

| Transformer oil with                                                        | 48 hours |            | 192 hours |            | 15 |
|-----------------------------------------------------------------------------|----------|------------|-----------|------------|----|
|                                                                             | Color    | Acid value | Color     | Acid value |    |
| No inhibitor                                                                | 2.5      | 22.5       |           |            |    |
| 0.05% dibenzyl disulfide                                                    | 1.5      | 0.04       | 4.5       | 0.25       |    |
| 0.10% dibenzyl disulfide                                                    |          |            | 8.0       | 0.25       |    |
| 0.005% 2,2' dihydroxy 1,1' dinaphthyl sulfide                               | 1.2      | 6.45       |           |            | 20 |
| 0.010% 2,2' dihydroxy 1,1' dinaphthyl sulfide                               | 1.5      | 10.00      |           |            |    |
| 0.05% dibenzyl disulfide plus 0.005% 2,2' dihydroxy 1,1' dinaphthyl sulfide | 0.8      | 0.02       | 3.5       | 0.13       |    |

Example 2.—Transformer oil, Coastal distillate, 50 lbs. of 98% and 100 lbs. of 104% sulphuric acid, neutralized and filtered, color less than 0.1; specific gravity 0.876; viscosity at 100° F., 56 sec.

| Transformer oil with                                                                | 48 hours |            | 96 hours |            | 192 hours |            | 35 |
|-------------------------------------------------------------------------------------|----------|------------|----------|------------|-----------|------------|----|
|                                                                                     | Color    | Acid value | Color    | Acid value | Color     | Acid value |    |
| No inhibitor                                                                        | 11       | 15.20      | 13       | 0.13       | 23        | 0.22       |    |
| 0.05% dibenzyl disulfide                                                            |          |            | 7        | 0.11       | 19        | 0.14       |    |
| 0.10% dibenzyl disulfide                                                            |          |            | 5.3      | 10.70      |           |            | 40 |
| 0.005% 2,2' dihydroxy 1,1' dinaphthyl sulfide                                       |          |            | 8.5      | 6.65       |           |            |    |
| 0.010% 2,2' dihydroxy 1,1' dinaphthyl sulfide                                       |          |            | 6.5      | 0.04       | 14        | 0.07       |    |
| 0.05% dibenzyl disulfide plus 0.005% 2,2' dihydroxy 1,1' dinaphthyl sulfide         |          |            | 14       | 6.05       |           |            | 45 |
| 0.010% monosulfide of m-cresol                                                      |          |            | 2.5      | 0.02       | 9         | 0.09       |    |
| 0.05% dibenzyl disulfide plus 0.005% monosulfide of m-cresol                        |          |            | 1.0      | 0.02       | 1.5       | 0.02       | 50 |
| 0.05% dibenzyl disulfide plus 0.010% monosulfide of m-cresol                        |          |            | 1.1      | 0.02       | 18        | 15.20      |    |
| 0.01% monosulfide of thymol                                                         |          |            | 7        | 0.08       | 17        | 0.15       |    |
| 0.05% dibenzyl disulfide plus 0.01% monosulfide of thymol                           |          |            | 1.7      | 0.02       | 4         | 0.07       | 55 |
| 0.05% dibenzyl disulfide plus sat. (approx. 0.005%) 4,4' dihydroxy diphenyl sulfide |          |            |          |            |           |            |    |

Example 3.—Turbine oil treated with 50 lbs. of 98% and 150 lbs. of 104% sulphuric acid per barrel of oil, neutralized and filtered. Color, less

than 0.1; specific gravity, 0.862; viscosity at 100° F., 122 sec.

| 5  | Inhibitor added                                               | 96 hours |            | 102 hours |            |
|----|---------------------------------------------------------------|----------|------------|-----------|------------|
|    |                                                               | Color    | Acid value | Color     | Acid value |
| 10 | 0.05% dibenzyl disulfide                                      | 14       | 0.16       | 22        | 0.24       |
|    | 0.05% dibenzyl disulfide plus 0.005% monosulfide of m-cresol  | 0.6      | 0.02       | 1.5       | 0.02       |
|    | 0.05% dibenzyl disulfide plus 0.0025% monosulfide of m-cresol | 6.0      | 0.07       | 14        | 0.20       |

- We have found that, in general, the optimum quantity of dibenzyl disulfide for stabilizing a highly refined viscous oil against color and acid formation is approximately 0.10% by weight or less, that is, that the use of any larger quantity imparts little or no greater stability to the oil.
- 20 In the case of the hydroxy-aromatic monosulfides, the optimum quantity is usually between 0.005% and 0.010%. It is evident, therefore, that the disproportionate result secured by the combined use of the two constituents in their optimum quantities or less, is due not to an increase in the total quantity of inhibiting material, but to some interaction or action in combination of the constituents.
- 25 In the aforesaid application, Serial No. 543,396

we have disclosed that the disulfides of organic compounds in general, and particularly of dialkyl compounds, are effective as stabilizers of highly refined viscous oils. Our experiments have indicated, however, that such disulfides do not have, in general, the peculiar cooperative relation with the hydroxy-aromatic monosulfides herein set forth. So far as we have ascertained, it is only in the case of dibenzyl disulfide that any notable increase in stabilization is secured by the inclusion of a hydroxy-aromatic monosulfide.

It will be understood that when we refer to a highly refined oil we intend an oil, however produced, which has essentially the same character as a heavily acid-treated oil, including a pronounced tendency to acidic oxidation.

We claim as our invention:

The combination, with a highly refined viscous mineral oil, of an addition of not over 0.10% dibenzyl disulfide and of substantially .005 to 0.010% of a substance of the class consisting of monosulfide of m-cresol, monosulfide of thymol, 2,2' dihydroxy, 1,1' dinaphthyl sulfide and 4,4' dihydroxy diphenyl sulfide, said addition being effective to stabilize said oil to a substantial degree, against acid formation.

BERTRAND W. STORY.  
EVERETT W. FULLER.